

## UNITED STATES PATENT OFFICE

2,039,595

METHOD OF TREATING HYDROCARBON  
MOTOR FUELS

Julius Hyman and George W. Ayers, Jr., Chicago,  
Ill., assignors, by mesne assignments, to Gaso-  
line Antioxidant Company, Wilmington, Del.,  
a corporation of Delaware

No Drawing. Application January 18, 1930,  
Serial No. 421,866

3 Claims. (Cl. 44-9)

This invention relates to hydrocarbon oils, particularly to those oils having relatively low boiling points and suitable for use as motor fuels. More specifically, the invention pertains to motor fuels produced by pyrogenic treatment of higher boiling oils, whereby the latter are split or cracked into similar compounds having approximately the boiling range of gasoline. Many cracked gasolines upon being exposed for some time to air, form 5 resinous materials which may be dissolved by the oil or may form insoluble deposits. These resinous compounds are formed particularly in large amounts in gasoline produced by vapor phase cracking, which gasolines contain a large 10 percent of unsaturated compounds. When such gasolines are exposed, under ordinary conditions of commercial handling, to heat, light and air, such unsaturated hydrocarbons react rapidly in producing the aforesaid gums or undesirable 15 resinous products. If the latter are permitted to form and remain in the motor fuel they are apt to interfere with the proper flow of the fuel through the restricted passages of internal combustion engines by producing deposits of such 20 gums in said passages to an extent sufficient to clog or obstruct the passages against the free or proper flow of the fuel to the combustion cylinders.

It is, therefore, an outstanding object of the 25 present invention to provide a cracked hydrocarbon motor fuel to which are added compounds, which for convenience in description may be termed "negative catalysts" or "gum inhibitors", 30 which will arrest for all practical purposes the formation of the objectionable resinous or gum compounds in the motor fuel product to the end that the latter may be subjected to the conditions prevailing in the storage, transportation and han- 35 dling of motor fuels without any appreciable development or formation of the objectionable gum substances in the fuel.

This application is a continuation in part of 40 our earlier application Serial No. 309,685, filed 45 October 1, 1928.

It has been discovered that certain substances when added to cracked petroleum gasolines retard the rate of formation of these resinous products. When p-aminophenol is added to a motor fuel oil containing unsaturated compounds, gum formation in such oils will be prevented substantially entirely under ordinary conditions of handling and storage for periods of several months.

The following table discloses results of gum

tests on vapor phase gasoline to which various anti-gum compounds have been added:

|               | Begin | 66 days | 96 days | 230 days | 400 days |
|---------------|-------|---------|---------|----------|----------|
| Blank         | .0010 | .0369   | .0609   | .0594    | .2521    |
| p-Aminophenol | .0010 | .0012   | .0013   | .0010    | .0014    |

From the foregoing it will be seen that by the 5 addition of p-aminophenol to cracked motor fuels, particularly fuels containing large percentages of unsaturated compounds, the fuels are stabilized for all practical purposes in so far as the formation of gum compounds is concerned. This 10 discovery is of far reaching importance in the manufacture of synthetic or cracked gasolines. The tendency at the present time in the manufacture of motor fuels is to produce motor fuels having a high anti-knock value, and such fuels 15 readily produce gums when exposed to light and air under ordinary conditions of handling, even after careful purification treatment with fuller's earth and similar polymerizing processes. The preferred method of treating such oils consists 20 in passing the cracked oils obtained directly from a cracking system while in a vaporous state into contact with a polymerizing catalyst such as fuller's earth, which accelerates the formation of 25 the polymers or gum compounds to permit of the removal of the latter to a very large extent from 30 the oils at the time the latter are manufactured. Then to prevent further formation of gums in the purified or polymer-free oils, the present 35 invention employs as a gum inhibitor p-aminophenol, which may be added in relatively small quantities, substantially ten pounds per thousand barrels of the cracked distillates to overcome further gum formation during ordinary handling, storage and transportation of the fuel. This insures delivery to the ultimate consumer of a gum-free motor fuel which will not produce resinous 40 deposits in the small fuel passages of an internal combustion engine or associated parts, and especially permits of the use of a pure hydrocarbon 45 motor fuel possessing high anti-knock value without the presence of objectionable and obnoxious gum deposits.

What is claimed is:

1. The method of preparing substantially gum-free and gum-stable motor fuel from vapor phase 50 cracked mineral oil which consists in contacting cracked oils boiling within the gasoline range with selective polymerizing catalyst under temperature and pressure conditions to maintain a substantial portion of said oils in vapor phase in order to re- 55

move gum and gum forming constituents and then adding to the degummed oil a small quantity of gum inhibitor sufficient to inhibit further formation of gum.

5. 2. Method in accordance with claim 1 in which the inhibitor is an amino-phenol capable of inhibiting gum formation in cracked gasoline.

3. The method of preparing substantially gum-free and gum-stable motor fuel from vapor phase  
10 cracked mineral oil which consists in contacting

cracked oils boiling within the gasoline range, at temperatures sufficiently high to maintain said oils in the vapor phase, with a selective polymerizing catalyst in order to remove gum and gum-forming constituents, and then adding to the degummed oil a small quantity of gum inhibitor sufficient to inhibit further formation of gum.

JULIUS HYMAN.  
GEORGE W. AYERS, JR. 10